

# UNITED STATES PATENT OFFICE.

EDWARD M. DAVIDSON, OF NEW YORK, N. Y., ASSIGNOR TO PYRENE MANUFACTURING COMPANY, A CORPORATION OF DELAWARE.

## PROCESS OF MAKING A FIRE-EXTINGUISHING COMPOUND.

1,036,461.

Specification of Letters Patent. Patented Aug. 20, 1912.

No Drawing. Original application filed April 5, 1910, Serial No. 553,570. Divided and this application filed December 4, 1911. Serial No. 863,939.

*To all whom it may concern:*

Be it known that I, EDWARD M. DAVIDSON, a citizen of the United States, and resident of the city, county, and State of New York, have invented certain new and useful Improvements in Processes of Making a Fire-Extinguishing Compound, of which the following is a specification.

This invention relates to a process of making a fire extinguishing compound having novel qualities which render it extremely efficient in extinguishing any ordinary fires and also results in the production of a compound which will successfully extinguish other extremely hot or refractory fires, either flaming or smoldering, by reason of its peculiar properties of establishing over the burning material a heavy, cohering, lingering and penetrating blanket of dry combustion arresting gas which effectually smothers and extinguishes the fire.

A further object of the invention is to provide a process of making an electrically non-conducting fire extinguishing compound which possesses all of the novel and peculiar properties above set out and in addition may be used on electrical fires. This compound is itself a non-conductor and when volatilized by the heat of the fire throws down a thick, gummy and electrically non-conducting deposit, which, when the fire is caused by a short circuit or the like, not only extinguishes the fire but prevents the reestablishment of the arc.

This application is a division of my application for a compound, filed April 5, 1910, Ser. No. 553,570.

The process of making this latter compound is similar to that for making the former, consisting in the addition of certain elements which add to the electric resistance of the compound and cause the non-conducting deposit to be thrown down when the compound is volatilized.

The improved compound, in its preferred form, has for its main ingredient a substance like carbon tetrachlorid, which volatilizes at temperatures encountered in fires to be extinguished, producing large volumes of heavy, penetrating gas. This carbon tetrachlorid contains ammonia gas and carbon dioxide gas in solution, sufficient carbon

dioxide being employed to form a saturated solution at or very slightly above atmospheric pressure. The liquid compound also contains when desired an electrically non-conducting ingredient, or ingredients, such as oil of amber and nitrobenzol, known as oil of mirbane, which add to the electrical resistance of the liquid and, in use, are thrown down on the burned material as a thick, gummy, electrically non-conducting deposit.

This compound may be formed by taking a quantity of carbon tetrachlorid and adding 1½% by volume of oil of amber and the same quantity of nitrobenzol, then passing 15% by volume of anhydrous ammonia gas into the solution under pressure, agitating the solution, passing approximately 22% by volume of anhydrous carbon dioxide into the solution under pressure and again agitating the solution, causing a complete chemical reaction in which the original ingredients are entirely changed.

The agitation of the solution may be accomplished by introducing the gas under a pressure sufficient to cause a complete mixing of the ingredients or, if this is not sufficient, any other suitable means may be employed, such as stirring, etc.

Applicant does not wish to be understood as limiting his invention to the specific ingredients herein set out as illustrative of a preferred embodiment of his invention, as it may be possible to substitute other ingredients or to vary the compound as defined in the appended claims without departing from the spirit of the invention.

What I claim is:

1. The process of making a fire extinguishing compound consisting in taking a quantity of carbon tetrachlorid and passing anhydrous ammonia gas into the same under pressure, agitating the solution, then passing anhydrous carbon dioxide into the solution under pressure, and again agitating the solution.

2. The process of making an electrically non-conducting fire extinguishing compound consisting in first forming a solution of carbon tetrachlorid with oil of amber and nitrobenzol and passing anhydrous ammonia gas into the same under pressure.

22  
agitating the solution, then passing anhydrous carbon dioxide into the solution under pressure, and again agitating the solution.

3. The process of making a fire extinguishing compound consisting in taking a quantity of carbon tetrachlorid and passing anhydrous ammonia gas into the same under pressure, agitating the solution, satu-

rating the solution with carbon dioxid gas and again agitating the solution.

Signed in the city, county and State of New York, this 29th day of November, 1911.

EDWARD M. DAVIDSON.

Witnesses:

OTTO KELSEY,

LEWIS J. DOOLITTLE.